

[54] **PROCESS OF MAKING HIGH STRENGTH COLD ROLLED STEEL HAVING EXCELLENT BAKE-HARDENING PROPERTIES**[75] Inventors: **Kuniki Uchida; Kenzi Araki; Hiroshi Narita; Shiro Fukunaka; Takao Kurihara**, all of Yokohama, Japan[73] Assignee: **Nippon Kokan Kabushiki Kaisha**, Tokyo, Japan[22] Filed: **July 11, 1974**[21] Appl. No.: **487,653**[30] **Foreign Application Priority Data**

July 12, 1973 Japan..... 48-77865

[52] U.S. Cl. .... **148/12.3; 148/12 F**[51] Int. Cl. .... **C21d 1/00**[58] **Field of Search** ..... 148/12 R, 12 C, 12 F, 12.3[56] **References Cited**

## UNITED STATES PATENTS

3,666,452 5/1972 Korchynsky et al..... 148/12 F  
3,666,570 5/1972 Korchynsky et al..... 148/12 F3,671,336 6/1972 Korchynsky et al..... 148/12 F  
3,787,250 1/1974 Korchynsky et al..... 148/12 FPrimary Examiner—W. Stallard  
Attorney, Agent, or Firm—Flynn & Frishauf[57] **ABSTRACT**

A high tension steel of which the yield point is more increased by the ensuring heat treatment after press-forming than that of the properties in which the tensile strength is above 40 to 80  $\text{Kg/mm}^2$ , is made by the following steps;

1. the chemical composition of steel is substantially controlled at the range of 0.04 to 0.12% C and 0.1 to 1.60% Mn,
2. the above steel is hot-rolled with a finishing temperature of more than  $800^\circ\text{C}$  and a coiling temperature of less than  $700^\circ\text{C}$ ,
3. after the above steel strip cold-reduced with the ordinary requirements is continuously heated up to  $700^\circ$  to  $900^\circ\text{C}$  and then rapidly cooled by a jet of water, said strip is reheated up to  $180^\circ$  to  $400^\circ\text{C}$  and held for 2 to 300 seconds at said temperature to partially remain solution carbon in steel.

5 Claims, 1 Drawing Figure





PROCESS OF MAKING HIGH STRENGTH COLD  
ROLLED STEEL HAVING EXCELLENT  
BAKE-HARDENING PROPERTIES

The present invention relates to a process of making an inexpensive high tension cold-reduced steel, and more in particular a process of offering cold-reduced steel excellent in accelerated aging properties wherein remarkable improvement in strength is seen by maintaining the tensile strength of 40 to 80 Kg/mm<sup>2</sup> and particularly, further increasing its yield point by the coming heat treatment after press forming in actual use.

Heretofore, it was well known in the art that the development of cold-reduced steel had been oriented toward a so-called soft steel having low yield point. In the process of pursuing safety in vehicles, however, particularly in passenger cars, the recent demand is oriented toward the cold reduced steel with high tensile strength. Various other proposals have been made and put into practice with this point in mind, and they may roughly be classified into the following:

1. That which performs a complete recrystallization by using special elements as Ti, Nb, Cu, Ni, etc.
2. That which controls the annealing requirements and partially retains the cold working structure.
3. That which re-cold-reduces the steel having completed recrystallization and tries to increase strength by work hardening.
4. That which aims at improving strength by quenching the low carbon steel.

It is true that these processes are defective in one way or the other. For instance, the process (1) is defective in its high cost, while the process (2) causes dispersions in the longitudinal direction as the differences in the annealing temperature occur in the inner and the outer peripheries of the coil. The process (3) does improve the strength, but its elongation is not improved proportionately, thus leaving a problem unsolved. On the other hand, the process (4) is suitable for obtaining inexpensive high tension cold-reduced steel and various proposals have been made recently in succession on said process, namely in Japanese Pat. Nos. 40-3020, 46-9541 and 46-9542.

The art disclosed in Japanese Pat. No. 40-3020 is well known as a BISRA process (in England). The art heats up the cold-reduced strip to 740° to 850°C, quenches the strip down to 150° to 250°C, coils the same and then performs an overaging treatment through self-annealing of said coil. The steel manufactured by said process has no accelerated aging property, i.e., AA property, caused by the heat treatment such as baking the coat after press forming, which causes an excessive lowering of the strength. Accordingly, it becomes necessary to further increase C content if the strength is to be enhanced. At the same time, the continuous process is interrupted by the above mentioned self-annealing, consequently decreasing the productivity.

Those arts disclosed in Japanese Pat. Nos. 46-9541 and 46-9542 are called the INLAND process (In America). The former heats up the coil comprising fine cementite or granular cementite and ferrite to more than the A<sub>3</sub> point in order to make perfect austenite structure not containing terminated pearlite, and then quenching uniformly to obtain a structure substantially comprising martensite. The latter heats up the coil from the A<sub>1</sub> to the A<sub>3</sub> point to obtain partial austenitiza-

tion, and then uniformly quenches the same to obtain the mixed structure of ferrite and martensite. The steels made by these processes are defective in that their strength is lowered by about 15 Kg/mm<sup>2</sup> by the coating and its baking after press forming, and that it has a poor ductility compared to its strength. This means that the steel is very difficult to handle since it is hard when being subjected to press forming and then it becomes soft when finished.

On the contrary, the steels excellent in the above AA property, which said strength is improved by the heat treatment after press forming, were proposed by the INLAND Steel Corporation. ("Blast Furnace and Steel Plant," March 1971, pp. 149 to 153). The art adds about 100 ppm nitrogen specially at the time of the initial steel-making stage. Such a steel is cold-reduced by the ordinary method, annealed by batch type annealing and then shipped. The users are expected to perform suitable press forming and a heat treatment to improve the strength. Such an improvement in strength is attributable to the aging of said nitrogen as above discussed, but it is true that such an effect is unfortunately limited automatically so that the initial strength is as low as 40 to 50 Kg/mm<sup>2</sup> in respect of its tensile strength while said AA effect is also as low as 5 to 6 Kg/mm<sup>2</sup>, thus imposing limitations in the applicable field of use. It may be said, therefore, that there is no process available today in the art which would obtain stable AA effects at the yield point of about 9 Kg/mm<sup>2</sup> at the baking stage after press forming.

The present invention was developed specifically to offer a solution comprising a method for overcoming the aforementioned difficulties and it is mainly characterized in that the manufacture is carried out by a continuous annealing process. Heating and soaking in this art is selected from among the range of 700° to 900°C at which the solution treating of cold-reduced steel is achieved, and the steel is subjected to quenching by a jet stream of water from the above temperature to the room temperature, then said steel is reheated to 150° to 400°C and is given the aging treatment at the said latter temperature. This aging treatment is not for completing the precipitation of C in the steel, but for causing partial remaining solution carbon therein. The steel is then cooled down to the room temperature and then coiled. After tempering, the tensile strength of 40 to 80 Kg/mm<sup>2</sup> is stably obtained. When the steel sheet thus obtained is subjected to the heat treatment for baking coat of said steel after press forming, its yield strength is improved by about 7 to 11 Kg/mm<sup>2</sup> in comparison with the initial strength before press-forming.

Thus, an object of this invention is to provide a process for manufacturing high tension steel sheet imparting safety to vehicles when used therein by improving of the accelerated aging property of said sheet.

Another object of this invention is to provide an inexpensive manufacturing process in a continuous annealing furnace of a high tension steel sheet excellent in accelerated aging property without addition of any special element.

Other objects and advantages will be apparent from the following description and with the accompanied drawing in which;

The FIGURE is a graph showing the variation of accelerated aging property dependent to the pre-heating requirements of travelling strip.

The steel to which the present invention may be applied consists of substantially 0.04 to 0.12% C and 0.10

o 1.60% Mn. There is no need for addition of special elements. Any type of furnace for manufacturing steel known in the art today may be used for this invention and any preferred processes after steel manufacture may be employed including ingot making — blooming, continuous casting, etc. After scarfing the steel is heated up to about 1,250°C or more, and is hot rolled at the finishing temperature of 800°C or more and a soiling temperature of 700°C or less. Ordinary cold reducing process may be employed after pickling. The annealing in the ensuing step is a complete continuous annealing process. In this case, said strip is heated up to 700° to 900°C and is maintained for 10 to 120 seconds at said temperature. The heating temperature should preferably be A<sub>1</sub> to 850°C and should be controlled rigorously since it will affect the strength of the final product very much.

C in steel thus made into solution in the above mentioned heating and soaking process. The following quenching from said temperature, should be performed as rapidly as possible. Therefore the use of a jet stream of water is recommended since C in steel will leave as solution carbon mentioned above. The travelling strip thus quenched down to the room temperature is reheated up to 150° to 400°C, and more preferably to 180° to 300°C and is to be maintained for some suitable length of time. The optimum period of maintaining depends on the reheating temperature, and more in particular the reheating temperature selected from among the range of 150° to 180°C will take 15 to 300 seconds; 180° to 300°C, 4 to 300 sec. or more preferably 20 to 120 sec.; and 300° to 400°C, 2 to 200 sec. This type of low temperature aging treatment will not cause the above-mentioned solution carbon in steel to precipitate completely but to remain partially in solution state. The travelling strip is then forcibly cooled down to the room temperature, coiled and tempered. The steel sheets thus obtained will easily have the following properties:

Tensile strength: 40 to 80 Kg/mm<sup>2</sup>

Yield strength: 30 to 60 Kg/mm<sup>2</sup>

Tensile strength (kg/mm<sup>2</sup>) + elongation (%): more than 73.

The value of TS (kg/mm<sup>2</sup>) + EI (%) is used as an index to evaluate the balance between the two since the increased strength usually lowers the elongation which represents ductility. The present invention steel thus treated will bring a remarkable improvement in the strength, particularly in the yield point of at least 7 Kg/mm<sup>2</sup> when given the heat treatment of 100° to 200°C after being pressed and formed into a shape intended. This naturally is attributable to the aging effects of the solution carbon partially left by the above-mentioned low temperature aging treatment. In other words, shaping is easily performed at the time of press forming because of the comparatively low yield point, consequently the excellent pressed shape of goods is maintained as it is, and the above-mentioned C aging effect becomes apparent in the baking process for said goods because of the heat used ordinarily performed to the goods thus shaped. This is none other but the object of the present invention, and the safety achieved when such a steel is used for passenger cars and the like, is unrivaled.

The present invention process is further elaborated in respect of its respective steps.

C in steel is an element which plays an important part in the present invention. Its lower limit is set at 0.04 percent in view of the stable operation of the converter used in most steel making stages and of the need to maintain required strength for steel. The upper limit was set at 0.12 percent in view of the press-formability and weldability. But more concretely, the upper limit should be selected from within the above range depending upon the levels of the required strength of steel. The lower limit of Mn content is set at 0.10 percent because of the red shortness. The upper limit thereof was set at 1.60 percent in view of the stable operations for the ingot making. Actually, Mn content is selected from within the range of 0.10 to 1.60 percent as is the case for determination of C content.

No undesirable effects are seen if Si and Al are maintained at 0.2 percent and 0.02 percent or less respectively in view of the deoxidation control. No specific limit is placed on P or S and they may be present at an ordinary level.

The hot rolling conditions for obtaining a uniform hot rolled structure should be such that the finishing temperature is more than 800°C and preferably 830°C or more. The cooling temperature may be on the same level as those for ordinary cold reduced sheets, that is below 700°C or 500° to 650°C on an industrial level. No special problems are existent if normal pickling and cold rolling after the hot rolling are performed.

The present invention is most remarkably characterized in its annealing process. The said annealing process is performed in one continuous line starting with paying-off of the cold rolled coils and finishing with coiling of annealed strip.

The heating requirements should be such that the strip must be heated up to a temperature where a great amount of solution carbon is formed in order to obtain the required strength since the hardening mechanism of the present invention steel depends greatly on the solution carbon in steel, fine precipitation therefrom and hardening thereby. That is to say, the heating-temperature should be at least 700°C or more and more than the A<sub>1</sub> point practically. On the other hand, the raising of said heating temperature in this way will increase quenching structure of martensite system thus increasing the strength of steel. However, this at the same time causes lowering of elongation since the differences of hardness between the ferrite matrix and the quenching structure as the second phase particles become larger. That is why there should be an upper limit imposed on the heating temperature such as 900°C at most and 850°C industrial-wise.

The minimum period of time for holding the travelling strip at the said heating temperature should be such that it will be sufficient for the cold rolled strip to complete recrystallization and for C in steel to become solution state. That is the reason for the lower limit of 10 seconds. However, the longer the holding time becomes, the more the softening acceleration caused by the grain grown after recrystallization occurs which at the same time requires extending of heating-soaking zone in the continuous treating line and lowering of the line speed. Thus the upper limit is placed at 120 seconds or less.

The travelling strip thus heated and soaked is quenched down to the room temperature by a jet stream of water. In this case, the jetting of water is used to speed up said cooling and display its full cooling effect irrespective of place, i.e., "in the air" or "under

water." That is to say, when the travelling strip heated is quenched into water, there is instantaneously produced a boiling steam film on the surface of said strip which damages the thermal conductivity and slows down the cooling speed excessively. The jet stream of water in this invention is the most useful in eliminating such a steam film and the applicants have proven through experiments that a high speed cooling of more than 3,000°C/sec. is easily obtained. On the other hand, it is confirmed that a cooling speed obtained by mere water, oil, salt bath or metal bath is only less than 1,000°C/sec. The reason for adopting such a high speed cooling rate in the present invention is because the solution carbon obtained through the process of heating and soaking is to be held there at room temperature. The quenching to the room temperature as above mentioned has determinative influences on the low temperature aging treatment which is the next step.

In reheating as the successive process of low temperature aging treatment as mentioned above, the precipitation nucleus for fine carbide of the solution carbon in steel is first formed. Fine carbide thus formed is quite useful for improving the strength, but will act to curb the lowering of strength caused by said solution carbon to a minimum. This is the first reason why the strip must be quenched down to the room temperature. The second reason is that if the steel was left as it was after being quenched to the room temperature, the strength at this stage due to solution hardening of C is extremely high. However, it is unavoidable that the above-mentioned solution carbon is precipitated and invites the lowering of strength by coating-baking treatment ordinarily performed after press forming (usually for 10 to 20 minutes at 100° to 200°C. In other words, it becomes most difficult to handle the steel since the strength is high at the time it is subjected to press-forming and becomes lower after press-forming. For this very reason, a low temperature aging treatment is performed by reheating the travelling strip that has been quenched down to the room temperature. In this stage, said solution carbon should be precipitated to a degree so as not to cause lowering of said strength at the time of coating-baking for formed goods. More concretely, the conditions for heating, soaking and cooling thereafter should be optimally provided for so that not all the solution carbon be precipitated by reheating, but some remain in solution state.

In the above-mentioned low temperature aging treatment, a good product with excellent AA property is obtained when the reheating temperature is low since the tensile strength will become higher and the yield strength lower as well as good shapability at the press forming stage. However, if the temperature is too low, there will occur no precipitation of solution carbon and the lowering of strength becomes unavoidable since said solution carbon is precipitated by the heat treatment in the coating-baking stage. Accordingly, the minimum reheating temperature is made at the temperature where the solution carbon is precipitated in part. The lower limit of such a temperature is 150°C. Concretely speaking, the temperature for treatment calls for above 180°C for obtaining stable results in view of the baking temperature after press forming.

On the other hand, too high a reheating temperature will soften a part of ferrite in the two phases structure wherein ferrite matrix and quenched structure coexist, thus causing inevitable lowering of steel strength. In addition, the differences in hardness between ferrite and quenched structure become remarkable so that there occurs no recovery of elongation in spite of the lowered tensile strength and the said "tensile strength + elongation" index becomes lower. High temperature reheating will also cause supersaturated solution carbon to precipitate in while at said aging treatment stage so that no AA effects can be anticipated. Accordingly, the upper limit of the reheating temperature is set at 400°C. There are no advantages obtained at the temperature exceeding 400°C. For practical purposes, the most preferable temperature is set at 180° to 300°C. The optimum range of the holding time for such reheating temperatures varies depending upon said temperature. If the said reheating temperature is set within the range of 150° to 180°C, the time should preferably be 15 to 300 seconds; if within 180° to 300°C, 4 to 300 seconds; if 300° to 400°C, 2 to 200 seconds respectively. If the said low temperature aging treatment is performed with such temperature  $x$  time requirements then all the problems that have been discussed heretofore will be dissolved, and it becomes easily feasible to cause some part of the solution carbon to remain in this stage. By such a process, the lowering of "tensile strength + elongation" index caused by the increased differences in hardness of the said two phase structure is possible to be avoided and sufficient AA effects are expected. In actual practice, when a holding time for 20 to 120 seconds as against a reheating temperature of 180 to 300°C is selected, the maximum AA properties, e.g.,  $\Delta YP$  is possible to be secured, which is recommended as the most suitable range. The graph in the accompanying drawing shows the fluctuation at this stage. It is seen at said graph that AA properties (in this case  $\Delta YP$  Kg/mm<sup>2</sup>) of at least 7 Kg/mm<sup>2</sup> are stably obtained when the temperature  $X$  time is selected from within the above range. It is possible to easily obtain the value of  $\Delta YP$  of 11 Kg/mm<sup>2</sup> with optimum conditions. In the said graph,  $\Delta YP$  shows the increase in yield point of the steels which have been subjected to the coating-baking process after press forming as versus those being just before said press forming.

There are no special restrictions imposed on the cooling requirements after the above mentioned low temperature aging treatment has been performed.

50 However, if forced air cooling should be employed because of the practical reasons, it is quite easy to cool the strip down to a temperature suitable for tempering in case that the temper rolling mill was connected integrally following the cooling step to the continuous line.

55 The strip is coiled off after temper rolling and is shipped out of the plant. If the said temper rolling mill were not to be attached, then a normal line of coiling the strip and then temper rolling the same is employed.

The following table shows the comparisons of the properties of this invention steels and those of other type steels.

| Steel | Composition |      |           | Heat treating requirements |              |            |             |
|-------|-------------|------|-----------|----------------------------|--------------|------------|-------------|
|       | C           | Mn   | Object    | Heating                    | Quenching    | Reheating  | Baking      |
| ° 1   | 0.07        | 0.39 | Influence | 800°C×1min                 | In jet water | 250°C×1min | 180°C×30min |

-continued

| Steel | Composition |      |                                       | Heat treating requirements |                    |             |        |
|-------|-------------|------|---------------------------------------|----------------------------|--------------------|-------------|--------|
|       | C           | Mn   | Object                                | Heating                    | Quenching          | Reheating   | Baking |
| 2     | "           | "    | of cooling method                     | "                          | In still water     | "           | "      |
| 3     | "           | "    |                                       | "                          | In 250°C lead bath | 250°C×1hr   | "      |
| 4     | "           | "    | Influence of max. heating temperature | 690°C×1min                 | In jet of water    | 250°C×1min  | "      |
| 5     | "           | "    |                                       | 750°C×1min                 | "                  | "           | "      |
| 6     | "           | "    |                                       | 800°C×1min                 | "                  | "           | "      |
| 7     | "           | "    |                                       | 850°C×1min                 | "                  | "           | "      |
| 8     | "           | "    |                                       | 920°C×1min                 | "                  | "           | "      |
| 9     | "           | "    | Influence of reheating temperature    | 800°C×1min                 | "                  | Non         | "      |
| 10    | "           | "    |                                       | "                          | "                  | 100°C×1min  | "      |
| 11    | "           | "    |                                       | "                          | "                  | 250°C×1min  | "      |
| 12    | "           | "    |                                       | "                          | "                  | 320°C×1min  | "      |
| 13    | "           | "    |                                       | "                          | "                  | 500°C×1min  | "      |
| 14    | "           | "    | Influence of reheating time           | "                          | "                  | 250°C×10sec | "      |
| 15    | "           | "    |                                       | "                          | "                  | 250°C×1min  | "      |
| 16    | "           | "    |                                       | "                          | "                  | 250°C×4min  | "      |
| 17    | "           | "    |                                       | "                          | "                  | 250°C×10min | "      |
| 18    | 0.07        | 0.39 | Influence of composition              | "                          | "                  | 250°C×1min  | "      |
| 19    | 0.10        | 0.45 |                                       | "                          | "                  | "           | "      |
| 20    | 0.15        | 0.37 |                                       | "                          | "                  | "           | "      |
| 21    | 0.07        | 0.58 |                                       | "                          | "                  | "           | "      |
| 22    | "           | 1.03 |                                       | "                          | "                  | "           | "      |
| 23    | "           | 1.52 |                                       | "                          | "                  | "           | "      |

(\* the present invention steels)

| T.S(Kg/mm <sup>2</sup> ) | After low temp. aging (1% skin pass) |                          |       | After baking |      |      | AA effects |        |  |
|--------------------------|--------------------------------------|--------------------------|-------|--------------|------|------|------------|--------|--|
|                          | Y.P(Kg/mm <sup>2</sup> )             | T.S(Kg/mm <sup>2</sup> ) | EI(%) | T.S+EI       | Y.P  | T.S  | Δ Y.P      | Δ T.S  |  |
| 68.1                     | 34.2                                 | 44.7                     | 30.9  | 75.6         | 44.5 | 45.5 | 10.3       | 0.8    |  |
| 55.0                     | 31.3                                 | 37.9                     | 28.6  | 66.5         | 36.3 | 37.8 | 5.0        | -0.1   |  |
| 49.5                     | 29.0                                 | 35.1                     | 33.3  | 68.4         | 32.1 | 35.0 | 3.1        | -0.1   |  |
| 54.8                     | 30.2                                 | 37.2                     | 35.0  | 72.2         | 35.2 | 37.0 | 5.0        | -0.2   |  |
| 61.3                     | 32.5                                 | 41.5                     | 33.0  | 74.5         | 42.0 | 42.8 | 9.5        | 1.3    |  |
| 68.1                     | 34.2                                 | 44.7                     | 30.9  | 75.0         | 44.5 | 45.5 | 10.3       | 0.8    |  |
| 65.2                     | 33.6                                 | 45.5                     | 27.5  | 73.5         | 43.2 | 45.5 | 9.6        | 0      |  |
| 65.5                     | 34.9                                 | 46.2                     | 21.7  | 67.9         | 42.6 | 46.0 | 7.7        | -0.2   |  |
| 68.1                     | —                                    | —                        | —     | 46.3         | 48.0 | —    | —          | -20.1① |  |
| "                        | 35.2                                 | 58.3                     | 15.8  | 74.1         | 45.3 | 47.5 | 10.1       | -10.8  |  |
| "                        | 34.2                                 | 44.7                     | 30.9  | 75.6         | 44.5 | 45.5 | 10.3       | 0.8    |  |
| "                        | 31.3                                 | 40.5                     | 32.9  | 73.4         | 39.2 | 40.0 | 7.9        | -0.5   |  |
| "                        | 26.5                                 | 35.5                     | 36.2  | 71.7         | 28.2 | 35.8 | 1.7        | 0.3    |  |
| "                        | 34.3                                 | 46.3                     | 28.5  | 74.8         | 45.2 | 45.7 | 10.9       | -0.6   |  |
| "                        | 34.2                                 | 44.7                     | 30.9  | 75.6         | 44.5 | 45.5 | 10.3       | 0.8    |  |
| "                        | 34.3                                 | 43.3                     | 30.0  | 73.3         | 41.2 | 43.6 | 6.9        | 0.3    |  |
| "                        | 33.5                                 | 41.1                     | 30.1  | 71.1         | 37.5 | 41.0 | 4.0        | -0.1   |  |
| 68.1                     | 34.2                                 | 48.7                     | 30.9  | 75.5         | 44.5 | 45.5 | 10.3       | 0.8    |  |
| 85.2                     | 37.1                                 | 50.2                     | 25.3  | 75.5         | 47.3 | 50.5 | 10.2       | 0.3    |  |
| 100.2                    | 46.2                                 | 59.3                     | 12.2  | 71.5         | 55.3 | 60.1 | 9.1        | 0.8    |  |
| 70.3                     | 36.5                                 | 46.3                     | 29.0  | 75.3         | 45.9 | 47.5 | 9.4        | 1.2    |  |
| 75.2                     | 48.2                                 | 63.3                     | 20.5  | 83.5         | 57.0 | 64.5 | 8.8        | 1.2    |  |
| 75.8                     | 50.5                                 | 65.0                     | 17.2  | 82.2         | 61.3 | 65.3 | 10.8       | 0.3    |  |

## Notes:

The requirements of manufacture other than those listed above are the same for all the steels and are as follows.

1. Hot rolling requirements: Finishing temperature: 850°C, cooling temperature: 600°C Finished thickness of strip: 2.8mm

2. Cold rolling requirements: Final sheet thickness: 1.2mm

3. Baking requirements after press forming are the same as those generally used in automobile manufacturing companies.

① Those compared with those after baking.

In the above table, the steels 1 to 3 were investigated in respect of the impacts of the cooling methods. The steel 1 was quenched in a jet water stream in accordance with the present invention. The steel 2 was quenched in still water and the steel 3 was quenched by BISRA method. The steel of the present invention shows the values of YP: 34.2 Kg/mm<sup>2</sup>, TS: 44.7 Kg/mm<sup>2</sup>, EI: 30.9 percent at the time of shipping out of the plant after skin pass; and the values of YP: 44.5 Kg/mm<sup>2</sup>, TS: 45.5 Kg/mm<sup>2</sup> after coating-baking treatment following press-forming indicating a remarkable improvement of ΔYP, namely by 10.3 Kg/mm<sup>2</sup>. This more than explains the excellent AA effects of the present invention and the reason for recommending the excellent quenching effects due to the jet water stream. The fact that "TS + EI" index in the present invention steel 1 is as high as 75.6 compared to 66.5 of the steel

55

60

65

2 and 68.8 of the steel 3 also suggests excellent press formability.

The steels 4 to 8 were investigated in respect of the impact of the maximum heating temperatures, and the steels 4 and 8 are comparison steels while the steels 5, 6 and 7 are the present invention steels. The maximum heating temperature is lower for the steel 4 than for the present invention steel while that for the steel 8 is higher conversely. The difference is clearly manifested in the mechanical properties of the steel. "YP + EI" index for comparison steels are all below 73 while those for the present invention steels exceed 73. This indicates that undesirable influences are seen in the press formability if the maximum heating temperature is outside the range of the present invention. This at the same time affects AA effects as illustrated by the fact that the present invention steels all show excellent ΔYP values of more than 9 Kg/mm<sup>2</sup> while the comparison steels

show quite insufficient values of 5.0 Kg/mm<sup>2</sup> and 7.7 Kg/mm<sup>2</sup> respectively. This fact tells that the desired objects are hardly achieved if the heating requirements are outside the range of the present invention even if the treatment following said quenching are the same.

Thus, the heating temperature should be selected from among the range of 700° to 900°C, and more preferably from A<sub>1</sub> point to 850°C.

The steels 9 to 13 were investigated in respect of the influences of reheating temperatures, and steels 9 to 10 and 13 are the comparison steels while steels 11 and 12 are the present invention steels. On these steels, the steel 9 was not given any reheating treatment, but shows remarkable lower value of TS, that is  $\Delta TS$  is as low as -20.1 Kg/mm<sup>2</sup> exemplifying a typical steel which is hard at the time of press forming and becomes soft as goods. Since the reheating temperature is 100°C for the steel 10, TS at the time of press forming is as high as 58.2 Kg/mm<sup>2</sup>. However, TS remarkably lowers to 47.5 Kg/mm<sup>2</sup>; i.e.,  $\Delta TS$ , to -10.5 Kg/mm<sup>2</sup> by the coating-baking after press forming and the steel is not a well balanced steel even if its  $\Delta YP$  showed 10.1 Kg/mm<sup>2</sup>. Thus, this steel 10 cannot be called one having good AA effects. Whereas, the steels 11 and 12 of the present invention maintain TS value as at the time of press forming while  $\Delta YP$  rises to 10.9 Kg/mm<sup>2</sup> and 7.9 Kg/mm<sup>2</sup> respectively and "TS + EI" index also show good values of 75.6 and 73.4 respectively. It is evident that the steels are well balanced and satisfactory. Thus, it is understood from the above going that the reheating temperature should be selected from within the range of 150° to 400°C and preferably 180° to 300°C.

The steels 14 to 17 were investigated in respect of the influences of a holding time at the reheating temperature. Of these steels, the steel 17 is the comparison steel while the steels 14 to 16 are the present invention steels. As shown in the table, the present invention steels 14 to 16 show well balanced properties and have sufficient AA effects. On the other hand, the comparison steel 17 with a long treatment time of 10 minutes have a low YP value of 4.0 Kg/mm<sup>2</sup>, thus displaying absence of AA effects. The holding time at reheating temperature is to be selected from within the range of 2 to 300 seconds, corresponding to the particular reheating temperature being employed.

The steels 18 to 20 were investigated in respect of the influences of the compositions, and the steel 20 is the comparison steel while the steels 18 to 19 are the present invention steels. The steel 20 has been subjected to identical treating requirements, except for its higher C content by 0.15 percent than the present invention steels. As is seen from the table, it has a low "TS + EI" index of 71.5. This clearly will present difficulties in stable formability and in weldabilities. Accordingly, the steel should be without doubt avoided even if it presents satisfactory AA effects after baking. On the other hand, the steels within the range of the present invention composition all show excellent "TS + EI" index and AA effects and are most satisfactory. Therefore, it becomes known that C content in steel should be within 0.12 to 0.04 percent range and should be varied depending upon the level of the strength required.

The steels 21 to 23 are the present invention steels and were investigated in respect of Mn influences. They show that the strength improved by Mn increase does not necessarily invite the lowering of elongation and does not invite the deterioration in "TS + EI" index. Thus, Mn is an effective element in the present in-

vention since it doesn't act to deteriorate the mechanical properties but improves the strength directly and its amount is selected according to the level of the strength required as in the case of determination of C content.

As has been explained in the above references being made to numerous examples, the fundamental technical differences as well as the remarkable effectiveness of the present invention method over the conventional BISRA process of semi-continuous process and the IN-LAND Steel process of batch type annealing aiming at AA effects by nitrogen in steel exist in; (1) the differences between quenching of the strip to coiling temperature in the lead bath in BISRA method and quenching down the strip to the room temperature in the jet water stream in the present invention method, (2) the differences of precipitation of solution carbon by self annealing at the said coiling temperature in BISRA process and the retaining of solution carbon caused by a reheating treatment in the present invention, and (3) the differences of the action of nitrogen content in the IN-LAND Steel type batch annealing where no aging effect caused by C content is possible and the controlling process solution carbon in the full continuous annealing process of the present invention (wherein N content is an unavoidable component in the steel making).

We claim:

1. In a process of making high strength cold-rolled steel sheet comprising a steel-making stage, a hot-rolling stage, a cold-reducing stage and a full continuous annealing stage, an improved process for obtaining a steel having excellent accelerated aging properties characterized in that:

1. at the above steel making stage, C content and Mn content in steel are controlled within the ranges of 0.04 to 0.12 percent and 0.1 to 1.60 percent respectively,

2. at the above hot-rolling stage, a finishing temperature of more than 800°C and a coiling temperature of less than 700°C are maintained,

3. at the full continuous annealing stage,

a. a travelling strip is heated up within the range of 700° to 900°C and is held at the above temperature for 10 to 120 seconds,

b. said heated and held strip is rapidly cooled by a jet stream of water to room temperature,

c. said rapidly cooled strip is reheated to the range of 150° to 400°C and held there for a period of time selected from the range of 2 to 300 seconds corresponding to the above reheating temperature, and

d. cooling and coiling the strip obtained in (c).

2. The process of claim 1, wherein said holding time at the reheating step of the full continuous annealing stage is from 15 to 300 seconds with said reheating temperature of 150° to 180°C.

3. The improved process as set forth in claim 1 wherein said holding time at the reheating step of the full continuous annealing stage is selected from the range of 4 to 300 seconds in case that said reheating temperature is set at the range of 180° to 300°C.

4. The improved process as set forth in claim 1 wherein said holding time at the reheating step of the full continuous annealing stage is selected from the range of 2 to 200 seconds in case that said reheating temperature is set at the range of 300° to 400°C.

5. The improved process as set forth in claim 1 wherein said holding time at the reheating step of full

continuous annealing stage is selected from the range of 20 to 120 seconds in case that said reheating temper-

ature is set at the range of 180° to 300°C.

\* \* \* \* \*

5

10

15

20

25

30

35

40

45

50

55

60

65

UNITED STATES PATENT AND TRADEMARK OFFICE  
CERTIFICATE OF CORRECTION

PATENT NO. : 3,904,446  
DATED : September 9, 1975  
INVENTOR(S) : KUNIKI UCHIDA et al

It is certified that error appears in the above-identified patent and that said Letters Patent are hereby corrected as shown below:

Column 1, line 10: before "strength", replace "is"  
with --- in ---.

Column 3, line 19: delete "ssteel";  
after "steel", insert --- is ---.

Columns 5-6, Table: under "Quenching", after "jet",  
insert --- of ---.

Column 10, line 24: Before "solution", insert --- of ---.

Signed and Sealed this  
second Day of March 1976

[SEAL]

Attest:

RUTH C. MASON  
Attesting Officer

C. MARSHALL DANN  
Commissioner of Patents and Trademarks